

June 21, 1932.

E. C. LOETSCHER

1,863,799

METHOD OF MAKING COATED ARTICLES

Original Filed Nov. 20, 1930

*Fig. 1.*



*Fig. 2.*



*Fig. 3.*



*Fig. 4.*



*Fig. 5.*



*Fig. 6.*



*Fig. 7.*



*Fig. 8.*



*Inventor:*  
Emil C. Loetscher,  
By Havell & Havell  
Atty's.

Patented June 21, 1932

1,863,799

# UNITED STATES PATENT OFFICE

EMIL C. LOETSCHER, OF DUBUQUE, IOWA

## METHOD OF MAKING COATED ARTICLES

Application filed November 20, 1930, Serial No. 496,988. Renewed February 15, 1932.

The object of this invention is to provide a method or process for making toilet seats, table tops, and various other articles from a fibrous material such as wood pulp, corn stalk pulp, bagasse, or any other elastic fibrous material, and covering the same with a synthetic resin.

Referring to the accompanying drawing, Fig. 1 is a perspective view of a closet seat.

Figs. 2, 3 and 4 are vertical sectional views taken on the line  $\alpha$ — $\alpha$  of Fig. 1, and illustrating various steps in the manufacture of a closet seat having a pressed pulp base.

Figs. 5, 6 and 7 are views similar to Figs. 2, 3 and 4 illustrating similar steps in the manufacture of a closet seat having a laminated base.

Figs. 8 and 9 are vertical sectional views illustrating the method of final coating and compressing the closet seat.

Referring to the drawing, reference numeral 15 designates an article produced under this invention, and while many articles may be made, including table tops and the like, a closet seat has been selected as the example. The article constructed may have a core or base 16 formed with an integral mass as in Figs. 2, 3, 4, 8 and 9 or may be formed with a laminated base 26, as in Figs. 5, 6 and 7. In constructing these bases the material is subjected to various degrees of compression until a very dense base product results, and this necessitates the selection of an elastic base material. This material may be wood pulp, corn stalk pulp, bagasse, or other similar fibrous material, with the fibers running in various directions to produce matting whereby a base structure is produced which is as strong, or even stronger than laminated wood, and less expensive.

In forming the base 16, a mass of one of the fibrous materials mentioned, as it comes from the beater, is placed in a pulp molding machine of the general type illustrated in Patent No. 827,815, dated August 7, 1906, and therein compressed to the general shape shown in Fig. 1, and the cross sectional shape illustrated in Fig. 2, the base being much thicker, though otherwise of substantially the same dimensions as it will be in its

final form. In this machine the desired quantity of water is extracted, though it may be necessary in some cases to subject the base to further pressure in a cooled press to remove the desired content of water to produce a preliminary but overthick base of compact mass. This base is then dried to remove substantially all of the water until it contains not over two per cent of moisture or less, producing the base 16 illustrated in Fig. 2.

This dried preliminary base 16 of Fig. 2 then receives a varnish coating 18 consisting of a solution of synthetic resin phenolic condensation product dissolved in alcohol, such as that known to the trade as bakelite varnish. This varnish coating penetrates the base about  $\frac{1}{2}$  of an inch. The outermost fibers are thoroughly coated and as they are criss-crossed in every direction, and in all planes, they produce a very good bond with the uncoated fibers of the interior of the base. This base is then placed in a drying inclosure at a temperature of approximately 110 to 120 degrees centigrade and dried until the alcohol is removed.

In making the laminated base 26 of Fig. 5, several fibrous boards or sheets, made from wood pulp, corn stalk pulp, bagasse or similar fibrous material, (the product known to the trade of "Cellotex" being well suited for the purpose) are glued together with a synthetic resin phenolic condensation product such as bakelite cement, though casein glue may be used. This adhesive, while coating the surfaces to be united, does not saturate the sheets, but only penetrates the same a slight distance, approximately  $\frac{1}{2}$  of an inch. This laminated stock is then cut out on a band saw, shaper or the like, to produce an overthick base corresponding in cross section to that of Fig. 8 and having the same dimensions thereas. The base 26 then receives a varnish coating at 28 in the nature of a solution of synthetic resin such as bakelite dissolved in alcohol, and known as bakelite varnish. The penetration of the coating 28 is the same in this case as that of the coating 18 in its case, and the following drying operation to remove the alcohol is the same.

55

60

70

75

80

85

90

95

100

Thus it will be seen that by the foregoing steps, there is produced a core base much thicker than, but otherwise of the same dimensions as the finally condensed base, and that such base has an exterior synthetic resin phenolic condensation product varnish coating which penetrates the base only approximately  $\frac{3}{8}$  of an inch, leaving the major portion of the interior of the base unsaturated and its compressibility unaffected. The core is now ready to receive its final exterior coating.

Heretofore, considerable difficulty has been experienced in producing core bases with pure white exterior coatings that will be virtually fire and water proof and resistant to the action of most alkalies and most acids. By the present method or process, the synthetic resin condensation product known as "Aldur" may be employed to advantage in securing the desired results. This product is made from formaldehyde and urea, though the latter may be replaced by theo-urea, and up to the present time has only been produced in powder form. It flows under heat and pressure and is not easily combustible and resists the action of alkalies, most acids, oils and practically all organic and inorganic solvents. In these characteristics it is superior to most synthetic resins and furthermore, being of pure white form, has the advantage of producing a pure white coating, mottled coating or coatings of all shades including black by the use of tints or dyes, whereas other synthetic resins being naturally of dark color (mostly brown) can only form coatings of dark shades.

In applying the final coating, and completing the compression of the base, the bottom of the cavity of a mold 30 is covered with enough of the selected synthetic resin 31 to make a final coating of approximately  $\frac{3}{8}$  of an inch in thickness on the bottom of the core or base. The previously shaped and coated base 16, (or 26 as the latter is under treatment), is then placed in the mold cavity, and a sufficient amount of the same synthetic resin (31) is applied to the upper surface of the base to give the same a final coating of approximately  $\frac{3}{8}$  of an inch in thickness and to join the coating material for the bottom of the base.

After the coating 31 has been applied to the base 16 (or 26) within the mold 30, the complementary mold section 35 is placed in position, and the whole mold assembly is placed in a hydraulic press. The press platens 36 and 37 are equipped with suitable means such as chambers 40 and 41 respectively for steam heating or water cooling. Rather high hydraulic pressure, ranging from 1,000 to 1,500 pounds per square inch of work area, is then applied, and while maintained, steam is circulated through the chambers 40 to maintain the mold and its contents for ap-

proximately five minutes. With the pressure maintained, the steam circulation is discontinued and water circulated through the chambers 41 for a few minutes to cool the mold and harden the coating 31 sufficiently to enable the article to be removed from the mold. Obviously instead of separate steam and water passages 40 and 41, these fluids may be circulated through the same chambers according to the type of press employed.

Care must be taken not to cool the mold too long, otherwise shrinkage of the coating will prevent removal of the article from the mold. Upon removal from the mold, the article will be found to have an exterior pure white coating of approximately  $\frac{3}{8}$  of an inch, incapable of being ignited below approximately 600 degrees, or of being scratched with one's finger nail, and having the stated qualities of being insoluble in most organic and inorganic solvents, or boiling water.

Bosses, lugs or other formations may be molded directly on to the article by suitable depressions in the mold parts 30 and 35 and with or without projections into these depressions, with room for the coating 30, of corresponding projections on the base 16 or 26.

The synthetic resin selected for the exterior coating 31, being produced up to the present time only in powdered form, does not, even when heated, have the penetrating effects of the material selected for the varnish coating 18 (or 28), and is more costly. The varnish coating, on the other hand, freely penetrates the fibrous material of the base the desired distance without saturating the same and under the heat treatment within the mold flows, as is also the case with the material of the coating 31, and forms a perfect union therewith. In other words by the use of the cheaper and more penetrating material employed for the coating 18 (or 28) the more expensive and less penetrating material employed for the coating 31 is caused to bond perfectly with the fibers of the base, and since both coating materials flow under heat and pressure, they offer no resistance to the final compression of the base.

It might be added, that the varnish coating 18 (or 28) because of its inherent dark color, is not applied in greater quantity than is essential to its proper functioning for the intended purpose, otherwise it will have a tendency, when mold heat and pressure are applied, to flow outwardly and penetrate the coating 30 to mar its appearance when being worked in white and certain lighter color shades.

It might also be stated that it is absolutely necessary to have the fibrous material compressible, as this produces a yielding surface and enables the material to conform to the shape of the mold or die, and without pene-

trating the exterior coating 31 to cause an imperfect product, as would be the case with incompressible base materials.

What is claimed:

- 5 1. The method of making a coated object, consisting in forming an oversize compressible base of matted fibers, varnishing the same with only slight interior penetration with a product that flows under heat and pressure, 10 applying a coating to the varnished base with a product that flows under heat and pressure, and then compressing the coated base to size under heat.
- 15 2. The method of making a coated object, consisting in forming an oversize compressible base of matted fibers, varnishing the same with only slight interior penetration with a synthetic resin that flows under heat and pressure and has penetrating characteristic, 20 applying a coating to the varnished base with a synthetic resin that flows under heat and pressure and has penetrating characteristic below that of the varnish, and then compressing the coated base to size under heat.
- 25 3. The method of making a coated object, consisting in forming an oversize compressible base of matted fibers, varnishing the surface of the same with only slight interior penetration with a synthetic resin that flows 30 under heat and pressure and has high penetrating characteristic, permitting the varnish to dry, applying to the varnished base a synthetic resin powder that flows under heat and pressure and has penetrating characteristic 35 below that of the varnish and which is capable of forming a bond with the varnish coating and is capable of producing alone a white coating or when tinted of producing black or intermediate color shades, and then compressing the double coated base to size under 40 heat.
4. The method of making a coated object, consisting in forming an oversize compressible base of matted fibers, varnishing the surface of the same with only slight interior penetration with a liquid synthetic resin phenolic condensation product that flows under heat and pressure and has high penetrating characteristic, permitting the varnish to dry, applying to the varnished base a synthetic resin condensation product of formaldehyde and a urea in powder form that flows under heat and pressure and has penetrating characteristic 50 below that of the varnish and which is capable of forming a bond with the varnish coating and is capable of producing alone a white coating or when tinted of producing black or intermediate color shades, and then compressing the double coated base to size 55 under heat.
- 55 5. The method of making a coated object, consisting in forming a compressible base of matted fibres, overthick but otherwise having approximately the same dimensions as it 60 will have when reduced to finished size; var-

nishing the same with only slight interior penetration and without major saturation with a product that flows under heat and pressure; applying a coating to the varnished base with a product that flows under heat and pressure; and then compressing the coated base to size under heat; the varnish coating being of a quantity insufficient to penetrate the outer coating when subjected to heat and pressure.

In testimony whereof I affix my signature.  
EMIL C. LOETSCHER.

70

75

80

85

90

95

100

105

110

115

120

125

130